



US006361225B1

(12) **United States Patent**  
Szajewski et al.

(10) **Patent No.:** US 6,361,225 B1  
(45) **Date of Patent:** Mar. 26, 2002

(54) **APPARATUS FOR PROVIDING A PHOTOCHEMICAL REACTION**(75) Inventors: **Richard P. Szajewski; Allan F. Sowinski**, both of Rochester, NY (US); **Nigel R. Wildman**, Watford (GB)(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/592,815**(22) Filed: **Jun. 13, 2000**(51) **Int. Cl.<sup>7</sup>** ..... G03D 5/00; G03D 5/06(52) **U.S. Cl.** ..... 396/604; 396/605(58) **Field of Search** ..... 396/604, 605, 396/606, 580, 33, 42(56) **References Cited**

## U.S. PATENT DOCUMENTS

|             |           |                  |         |
|-------------|-----------|------------------|---------|
| 2,558,857 A | 7/1951    | Land             | 396/33  |
| 2,848,931 A | 8/1958    | Troidl           | 396/575 |
| 2,880,657 A | * 4/1959  | Bartlett         | 396/605 |
| 2,930,302 A | * 3/1960  | Tuttle           | 396/605 |
| 3,179,517 A | 4/1965    | Tregillus et al. | 430/207 |
| 3,282,695 A | * 11/1966 | Narodny          | 396/606 |
| 3,419,006 A | 12/1968   | King             | 424/445 |
| 3,573,912 A | 4/1971    | Brown            | 430/346 |
| 3,615,482 A | 10/1971   | Cronig           | 430/404 |
| 3,664,343 A | 5/1972    | Assarsson        | 604/372 |
| 3,680,462 A | * 8/1972  | Cronig           | 396/606 |
| 3,907,563 A | 9/1975    | Land             | 430/206 |

|             |          |                   |                  |
|-------------|----------|-------------------|------------------|
| 3,993,551 A | 11/1976  | Assarsson et al.  | ..... 204/159.14 |
| 4,605,608 A | 8/1986   | Bullitt           | ..... 430/206    |
| 5,028,339 A | 7/1991   | Clark, III        | ..... 210/688    |
| 5,115,801 A | 5/1992   | Cartmell et al.   | ..... 602/48     |
| 5,378,542 A | 1/1995   | Hanzalik et al.   | ..... 428/483    |
| 5,440,366 A | * 8/1995 | Reiss et al.      | ..... 396/605    |
| 5,453,804 A | 9/1995   | Norris et al.     | ..... 396/31     |
| 5,714,159 A | 2/1998   | Shalaby           | ..... 424/426    |
| 5,792,471 A | 8/1998   | Curatolo          | ..... 424/180    |
| 5,840,471 A | 11/1998  | Fukuwatari et al. | ..... 430/399    |

## FOREIGN PATENT DOCUMENTS

|    |          |        |
|----|----------|--------|
| GB | 1121277  | 7/1968 |
| JP | 02-13947 | 1/1990 |

\* cited by examiner

Primary Examiner—D. Rutledge

(74) Attorney, Agent, or Firm—J. Lanny Tucker

(57) **ABSTRACT**

An apparatus can be used to process photographic silver halide materials in an “almost dry” format. This apparatus includes means for supplying the photographic material as well as photochemical delivery articles and means for providing the chemicals for photochemical reaction and image formation. The apparatus can also include heating means for speeding up the reaction, scanning means and solution applicators at various stations. The delivery articles can be laminated or otherwise contacted with the imaged photographic materials on the silver halide emulsion side allowing photochemicals to diffuse into and out of the materials for the desired chemical reactions. Multiple delivery articles can be used in sequence to provide the desired sequence of photochemical reactions.

27 Claims, 3 Drawing Sheets





FIG. 1



FIG. 2



FIG. 3

APPARATUS FOR PROVIDING A  
PHOTOCHEMICAL REACTION

## FIELD OF THE INVENTION

This invention relates to an apparatus for providing one or more photochemical reactions in imaging materials. In particular, this apparatus is useful to provide photochemical reactions in color or black-and-white photographic imaging materials using a novel photochemical delivery article comprising a hydrogel.

## BACKGROUND OF THE INVENTION

The basic image-forming process of photography comprises the exposure of a silver halide photographic recording material, such as a color film, to electromagnetic radiation, and the chemical processing of the exposed material to provide a useful image. Chemical processing involves one fundamental step and one or more ancillary steps. The fundamental step is treatment of the exposed silver halide material with a developing agent wherein some or all silver ion is reduced to metallic silver, and in the case of color materials, a dye image is formed (because of a color developing agent).

For color materials, ancillary steps include the removal of silver metal and silver salts by one or more steps of bleaching and fixing so that only a dye image remains in the processed material. These steps are commonly used to enable optical printing and can make scanning easier. During bleaching, the developed silver is oxidized to a silver salt by a suitable bleaching agent. The oxidized silver is then dissolved and removed from the material using a "fixing" agent or silver solvent in a fixing step. Black-and-white materials are desilvered using only the fixing step.

Additional photoprocessing steps may be needed including rinsing or dye stabilization that requires even more photoprocessing chemicals. In the case of color reversal materials, additional photoprocessing steps include black-and-white development, a reversal step, pre-bleaching or conditioning step and one or more rinsing steps.

All of these photoprocessing steps require preparation of the photoprocessing compositions (whether in aqueous or solid form), large or small photoprocessing tanks or reservoirs to hold the compositions, and disposal or regeneration of the "spent" compositions once a predetermined amount of exposed material has been processed. All of these operations require considerable manufacturing effort, shipping and handling of chemicals and aqueous solutions, replenishment of the solutions, and disposal of solutions into the environment. These characteristics of conventional photoprocessing are labor intensive, tedious, costly and potentially harmful to the environment (although much work has been accomplished in the industry to make the compositions more environmentally "friendly").

New business opportunities are thought to exist if ways can be found to minimize or obviate the problems described above. Providing photographic images (often known as "photofinishing") is a growing business and yet there is a need to provide those images in ways that do not require some or all of the traditional photoprocessing solutions, equipment and replenishment systems.

Various research efforts have been carried out in the industry to provide new methods of imaging. For example, research has been carried out directed at putting photoprocessing chemicals directly into the imageable materials. Coated donor/receivers systems on flexible supports have

been developed in recent decades for output media (such as color prints). The conventional "instant" photographic materials are examples of imaging materials that include coated and/or delivered photoprocessing chemicals. See for example, U.S. Pat. No. 4,605,608 (Bullitt).

U.S. Pat. No. 5,453,804 (Norris et al) describes a hydrogel, rolled flexible carried material that comprises an aqueous, alkaline processing composition that is used in an image transfer processing method. This material does not include a backing sheet or non-porous supporting substrate.

All of the ongoing research efforts still have some unattractive features pertaining to the delivery of the photoprocessing chemicals (identified as "photochemicals" hereinafter). To date, the need for enabling technology remains unsatisfied.

Photoprocessing webs comprised of gelatin or other hydrophilic colloids are also known as described for example in U.S. Pat. No. 3,179,517 (Tregillus et al).

In order to simplify the mechanical requirements of photoprocessing, it would be desirable to avoid high precision fluid spreading that may be required in extrusion hopper metering or a fluid bath for coating materials to be laminated. Thus, there continues to be a need for unique equipment or apparatus useful for photoprocessing that is not accompanied by the problems noted above with traditional methods or known research methods. It would also be useful to have such an apparatus that is adapted to process the images in an efficient and simple manner, but that also enables digitization of those images.

## SUMMARY OF THE INVENTION

An advance in the photographic art is provided with an apparatus for providing a photochemical reaction comprising:

- a) a means for supplying an imagewise exposed photographic silver halide material comprising at least one silver halide emulsion layer,
- b) a means for supplying a photochemical delivery article consisting essentially of a nonporous substrate having disposed thereon a hydrogel containing one or more diffusible photochemicals,
- c) a means for bringing the imagewise exposed photographic silver halide material and the photochemical delivery article into reactive association to form a web laminate so that a photochemical reaction can occur, and
- d) a downstream web laminate treating means that is either
  - i) a means for removing said nonporous substrate from the photochemical delivery article in the web laminate, or
  - ii) a means for delaminating the photochemical delivery article from the imagewise exposed photographic silver halide material, and a means for collecting the delaminated photochemical delivery article.

Another apparatus for providing a photochemical reaction comprises:

- a) a means for supplying an imagewise exposed photographic silver halide material comprising at least one silver halide emulsion layer,
- b) a means for supplying a photochemical delivery article consisting essentially of a nonporous substrate having disposed thereon a hydrogel containing one or more diffusible photochemicals, and
- c) a means for bringing the imagewise exposed photographic silver halide material and the photochemical

delivery article into reactive association to form a web laminate so that a photochemical reaction can occur. Further, an apparatus for providing a photochemical reaction comprises:

- a) a means for supplying an imagewise exposed photographic silver halide material comprising at least one silver halide emulsion layer,
- b) a means for supplying a photochemical delivery article consisting essentially of a nonporous substrate having disposed thereon a hydrogel that is substantially free of diffusible photochemicals,
- c) a means for bringing the imagewise exposed photographic silver halide material and the photochemical delivery article into reactive association to form a web laminate,
- d) a means for removing the nonporous substrate from the photochemical delivery article in the web laminate, and
- e) a means for supplying one or more diffusible photochemicals to the photochemical delivery article in the web laminate.

The present invention avoids the need for high precision fluid spreading required for extrusion hopper metering. It also avoids the traditional processing baths and equipment used in conventional photoprocessing and all the problems they entail.

These advantages are provided with the use of an apparatus in conjunction with a novel photochemical delivery article that can be laminated to imagewise exposed photographic silver halide materials to deliver photochemicals for image formation. This lamination operation allows diffusible photochemicals to move into and out of the imagewise exposed photographic materials for a period of time sufficient for desired photochemical reactions to occur. Once the method is finished, the contacted material needs little or no further handling.

The photochemical delivery article is a permeable matrix composed of a hydrogel that, in most embodiments, has been impregnated or swollen with one or more photochemicals prior to use. The article can be used to deliver the photochemicals in a controlled fashion to the same or different materials without additional fluid extrusion, pumping or dipping the materials into processing baths. Different delivery articles can be used in sequence to deliver the different photochemicals necessary for the various sequential photochemical reactions required for providing a color or black-and-white image. For example, in providing color negative images, one photochemical delivery article could be used to deliver a color developing agent and one or more other photochemical delivery articles can be used thereafter to desilver the material. Following all necessary processing steps and drying, the processed material either can have a viewable image or be used to provide a viewable image in any suitable fashion.

In some embodiments, the photochemical delivery article is substantially free of photochemicals when it is laminated to the processed photographic material. However, photochemicals can be delivered to the article while it is in the web laminate.

The hydrogel containing delivery articles are advantageous because they readily absorb solvents (containing needed diffusible photochemicals), undergo rapid swelling without discernable dissolution and maintain three-dimensional networks capable of reversible deformation while maintaining their physical and mechanical integrity. Thus, photochemicals can be imbibed into the matrices with minimal effort, and they can be readily absorbed into the imaged materials in the same manner.

The photochemical delivery articles used with the apparatus of this invention are described and claimed in copending and commonly assigned U.S. Ser. No. 09/593,097 filed on even date herewith by Sowinski, Szajewski and Wildman, entitled "Photochemical Delivery Article and Method of Use."

The apparatus of this invention can be used to advantage in the imaging methods described in copending and commonly assigned U.S. Ser. No. 09/593,089 filed on even date herewith by Sowinski, Szajewski and Wildman, entitled "Method of Providing Digitized Photographic Image."

#### BRIEF DESCRIPTION OF THE DRAWINGS

FIG. 1 shows an apparatus of this invention that uses a single photochemical delivery article to process a photographic material in a web laminate.

FIG. 2 shows an apparatus of this invention that uses two different photochemical delivery articles to process a photographic material.

FIG. 3 shows an apparatus of this invention that uses a single photochemical delivery article and several delivery stations for supplying an aqueous solution to a photographic material.

#### DETAILED DESCRIPTION OF THE INVENTION

The present invention is better understood by making reference to FIGS. 1-3 that illustrate several representative embodiments of this invention. It is to be understood however, that these embodiments are not the only ones within the present invention. Additional embodiments and details of the various apparatus would be readily apparent to one skilled in the art.

For example, an apparatus of this invention comprises:

- a) a means for supplying an imagewise exposed photographic silver halide material comprising at least one silver halide emulsion layer,
- b) a means for supplying a photochemical delivery article consisting essentially of a nonporous substrate having disposed thereon a hydrogel containing one or more diffusible photochemicals,
- c) a means for bringing the imagewise exposed photographic silver halide material and the photochemical delivery article into reactive association to form a web laminate so that a photochemical reaction can occur,
- d) a means for removing the nonporous substrate from the photochemical delivery article in the laminate,
- e) a means for scanning the web laminate to provide density representative signals, and
- f) a means for delaminating the photochemical delivery article from the imagewise exposed photographic silver halide material.

This embodiment of this invention is illustrated for example in FIG. 1. Imagewise exposed photographic silver halide material 12 ("photographic material") containing at least one silver halide emulsion layer is supplied as a web from camera spool 10 and taken up by accumulator 20. Optional dual guides 14, 16 and 18 serve to guide and constrain the material to the desired path through the apparatus. In most instances, this photographic silver halide material has been imagewise exposed using any suitable means for that purpose (for example, a camera). Photochemical delivery article 34 is supplied as a web from supply reel 22 in roll form and applied to photographic material 12 at roller 15 to form web laminate 11. Photochemical delivery

article 34 comprises nonporous substrate 36 that is peeled or otherwise removed from web laminate 11 at roller 17 to form substrate-free web laminate 13. The removed nonporous substrate 36 is taken up or collected on reel 24. The remaining hydrogel 38 is pulled away from substrate-free web laminate 13 at roller 19 and taken up or collected on reel 26.

Optional blades (not shown) can be positioned between roller 17 and dual guides 16 and between roller 19 and dual guides 18 as a means for removing nonporous substrate 36 and hydrogel 38, respectively, from the various web laminates.

Imagewise exposed photographic silver halide film 12 is processed to form a useful photographic image by contact with photochemical delivery article 34 as the laminates travel between rollers 15 and 19. Optional heating stations (not shown) can be located so as to heat web laminate 11 and/or substrate-free web laminate 13 if desired to quicken photochemical reaction. An optical cooling station (not shown) can also be positioned after any heating station to cool the film.

An electronic scanning station or means includes light source 28 that emits a beam of light 30 and sensor 32 that senses light passing through substrate-free web laminate 13 as it passes between roller 17 and accumulator 20. As described in more detail below, the scanning means provides density representative signals from the image in the photographic material, which signals can be used in various ways.

In one embodiment, photochemical delivery article 34 is contacted with water or an aqueous solution (such as a buffer, photochemical activator solution, photographic color or black-and-white developing solution or chemical base) before it is wound or collected on supply reel 22. For example, such aqueous solutions serve to promote processing (such as development) of imagewise exposed photographic material 12 while it is in contact with photochemical delivery article 34.

In another embodiment, camera spool 10 is a thrust cartridge and the drive for the thrust cartridge is coordinated with the drives for supply reel 22 and take-up reels 24, and 26. In this instance, accumulator 20 serves to store photographic material 12 until it is rewound into the thrust cartridge.

In still another embodiment, camera spool 10 is a standard film spool and accumulator 20 actively collects photographic material 12. In this instance, dual guides 14, 16 and 18 can be dual nib rollers that drive photographic material 12 through the apparatus. The web drives can be coordinated with the supply reel 22 and take-up reels 24 and 26. It is useful to coordinate the advance of a photographic material and the photochemical delivery article advance so as to minimize scratching of the photographic material surface while it is processed.

In still another embodiment, an apparatus for providing a photochemical reaction comprises:

- a) a means for supplying an imagewise exposed photographic silver halide material comprising at least one silver halide emulsion layer,
- b) a means for supplying a first photochemical delivery article consisting essentially of a nonporous substrate having disposed thereon a hydrogel containing a first diffusible photochemical,
- c) a means for bringing the imagewise exposed photographic silver halide material and the first photochemical delivery article into reactive association to form a first web laminate so that a first photochemical reaction can occur,

- d) a means for delaminating the first photochemical delivery article from the imagewise exposed photographic silver halide material,
- e) a means for supplying a second photochemical delivery article consisting essentially of a nonporous substrate having disposed thereon a hydrogel containing a second diffusible photochemical, and
- f) a means for bringing the imagewise exposed photographic silver halide material and the second photochemical delivery article into reactive association to form a second web laminate so that a second photochemical reaction can occur.

This apparatus for using multiple photochemical delivery articles in sequence is illustrated for example in FIG. 2. While this drawing illustrates the use of only two such articles, it would be readily apparent to a skilled artisan that an apparatus could be designed to utilize three or more such articles where photoprocessing requires a multiplicity of individual photoprocessing reactions.

The basic arrangement of components and stations on the left side of FIG. 2 (prior to dual guides 18) is similar to that shown in FIG. 1. Dual guides 52, 54 and 56 also serve to constrain photographic silver halide material 12 in the desired path through the apparatus. A second photochemical delivery article 46 is supplied in roll form from supply reel 40 and applied to photographic material 12 at roller 53 to form web laminate 49. Nonporous substrate 48 is peeled from web laminate 49 at roller 55 leaving substrate-free web laminate 51 and substrate 48 is taken up or stored on reel 42. The remaining hydrogel 50 is separated from material 12 in substrate-free web laminate 51 at roller 57 and taken up on reel 44. Optional peeling blades (not shown) can be positioned between roller 53 and dual guides 52 and between roller 57 and dual guides 56. The photographic material 12 is processed by contact with the two distinct photochemical delivery articles 34 and 46 between rollers 15 and 19, and 53 and 57, respectively. The two photochemical delivery articles can include the same or different photochemicals.

Alternatively, either or both delivery articles can be substantially free of photochemicals before being laminated. Photochemicals can be supplied to the hydrogel while it is in one of the web laminates.

Optional heating stations (not shown) can be located in the apparatus so as to heat the any or all of the web laminates between rollers 15 and 57. Optional cooling stations (not shown) can also be used to cool the processed photographic material at any position or station in the apparatus. In the illustrated embodiment of FIG. 2, an electronic scanning station or means includes light source 28 that emits a beam of light 30 and sensor 32 that senses light passing through photographic material 12 between roller 57 and accumulator 20. However, such a scanning means can be positioned anywhere in the apparatus, and multiple scanning means can be positioned at various stations in the apparatus, for example to scan any of the web laminates 11, 13, 49 or 51 as well as photographic material 12.

In other embodiments, photochemical delivery article 34 and/or 46 can be contacted with water or an aqueous solution (such as a buffer, photochemical activator solution, photographic color or black-and-white developing solution, chemical base, photographic bleaching solution, or photographic fixing solution) before it is wound onto supply reel 22 or 40, respectively. For example, such aqueous solutions serve to promote processing (such as development, bleaching or fixing) of photographic material 12 while it is in contact with the various photochemical delivery articles.

For example, photochemical delivery article 34 can be contacted with a developing composition, and photochemi-

cal delivery article 46 can be contacted with a bleaching and/or fixing solution to provide the sequential photochemical reactions used in many photoprocessing methods.

Still again, either or both of photochemical delivery articles 34 and 46 can be supplied free of photochemicals, but after lamination, they can be contacted with appropriate photochemicals.

Still another embodiment of this invention includes an apparatus comprising:

- a) a means for supplying an imagewise exposed photographic silver halide material comprising at least one silver halide emulsion layer,
- b) a means for supplying a photochemical delivery article consisting essentially of a nonporous substrate having disposed thereon a hydrogel containing one or more diffusible photochemicals,
- c) a means for bringing the imagewise exposed photographic silver halide material and the photochemical delivery article into reactive association to form a web laminate so that a photochemical reaction can occur,
- c') a means for contacting the imagewise exposed photographic silver halide material with an aqueous solution prior to its being laminated,
- d) a means for removing the nonporous substrate from the photochemical delivery article in the web laminate to form a substrate-free web laminate,
- d') a means for contacting the substrate-free web laminate after removal of the nonporous substrate with one or more aqueous solutions,
- e) a means for scanning the substrate-free web laminate to provide density representative signals, and
- f) a means for delaminating the photochemical delivery article from said imagewise exposed photographic silver halide material.

This embodiment is illustrated for example in FIG. 3 and is similar to the apparatus illustrated in FIG. 1 except for some additional components or stations. As shown in FIG. 3, an aqueous solution (such as a chemical base activator solution) can be applied to photographic material 12 from applicator 58 as shown by arrow 60. Photographic material 12 is treated similar as shown in FIG. 1 until nonporous substrate 36 is removed at roller 17. A second aqueous solution (such as a color or black-and-white developing solution) is applied from applicator 62 at arrow 64. Still another aqueous solution (for example an acidic "stop" solution) can be applied using applicator 66 at arrow 68. The remaining stations and features are the same as those described in FIG. 1.

The various "applicators" in FIG. 3 can be any suitable source of aqueous solutions including drip applicators, processing tanks or containers, lines from processing tanks or containers, "bubble-jet" or ink-jet type applicators.

Photochemical delivery article 34 serves to distribute the applied aqueous solution thereby suppressing drip and flow marks on the processed photographic material 12. In another embodiment, additional applicators are arranged to apply desilvering solutions (bleaching, fixing or bleach-fixing solutions) to the same or different photochemical delivery article prior to its use. When such desilvering solutions are employed, however, it can be advantageous to locate the scanning means so as to scan the processed photographic material 12 between roller 19 and accumulator 20.

In some embodiments, it may be desirable to include one or more heating means (heated platen, heated rollers, infrared heaters or gas heaters (in the apparatus to increase photochemical reaction time in the web laminates. Such

heating means can be located in various stations of the apparatus. For example, in reference to FIGS. 1-3, a heating means can be located between rollers 15 and 17, or between rollers 17 and 19 or between roller 19 and accumulator 20.

In addition, the apparatus can include a means for applying pressure to the various web laminates. Such pressure applying means can include pressure rollers (for example rollers 15 and 53 in FIGS. 1-3) or the nib rollers can be configured to apply pressure across the reactive surface of the web laminates.

The apparatus of this invention can be arranged as a system of individual components or stations that can be assembled or disassembled when desired. Alternatively, it can be a single piece of equipment with the desired stations and components integrated into a self-contained unit.

In still another embodiment of this invention, an apparatus includes a supply of one or more photochemical delivery articles that contain substantially no photochemicals. However, the photochemicals can be applied to the processed photographic material using other means, such as applicators like those shown in FIG. 3 above. While laminated to the processed photographic material, the photochemical delivery article is then used to spread or evenly distribute to the applied solutions of photochemicals.

The photochemical delivery articles useful in this invention contain only two essential structural components: a nonporous substrate and a hydrogel disposed thereon. The diffusible photochemicals (described below) are preferably incorporated within the hydrogel. Thus, there is no image-receiving or image-donating material or layer as described in U.S. Pat. No. 4,605,608 (noted above).

The nonporous substrate serves to provide some physical and mechanical integrity to the delivery article, and can be also considered a "backing sheet", support or release liner. It is preferred that the nonporous substrate be dimensionally stable, but remain flexible and deformable, allowing easy storage in roll form. Conventional photographic film supports and hydrogel wound dressing backing sheets are examples of useful support materials that have a desirable blend of plasticity and dimensional stability.

In one contemplated embodiment, the nonporous substrate is bonded to the hydrogel and is not releasable from it without force. This arrangement allows easy separation of the hydrogel from a laminate with a processed photographic material following the processing step. Alternatively and preferably, a removable substrate can be separated from the hydrogel to provide access to the top surface of the hydrogel-photographic material web laminate to allow application of additional fluids, processing solutions or activator solutions.

The substrate should be as thin as possible, for example, generally less than 500  $\mu\text{m}$  and preferably less than 200  $\mu\text{m}$ . The minimum thickness would depend upon the type of material composing the substrate but generally it is at least 75  $\mu\text{m}$ . The substrate is nonporous so the photochemicals more readily diffuse into the photographic material. In other words, the substrate acts as a fluid barrier and is therefore substantially fluid impermeable.

The substrate further serves to prevent the hydrogel from adhering to itself. The photochemical delivery article can be stored and used as sheets or strips. Preferably, it can be stored and used in roll form for use in the apparatus of this invention, and it is even more important that the hydrogel not adhere to itself in that form. In addition, the substrate would provide additional advantages of a barrier material to reduce air permeation or dehydration.

The substrate can be transparent and colorless, tinted or opaque to light depending upon the particular use of the photochemical delivery article.

The substrates can be homogeneous (same composition throughout) or heterogeneous (varying composition) and can be composed of synthetic or naturally-occurring polymeric materials, metal foils or flexible ceramics. Examples of useful substrate materials include, but are not limited to, resin-coated papers, polyethylenes, polypropylenes, polyethylenepolypropylenes, polyvinylidene chloride, polyamides, polyesters (such as polyethylene terephthalate and polyethylene naphthalate), polyvinyl chloride, cellulosic polymers (such as cellulose triacetate), polyurethanes, polyvinyl alcohol, silicone rubbers, polyvinyl (meth)acrylates, polystyrenes and others too numerous to mention. Other useful substrate materials are those used in conventional photographic materials as described for example in *Research Disclosure*, publication 38957, pages 592-639 (September 1996) Section XV Supports. *Research Disclosure* is a publication of Kenneth Mason Publications Ltd., Dudley House, 12 North Street, Emsworth, Hampshire PO10 7DQ England (also available from Emsworth Design Inc., 121 West 19th Street, New York, N.Y. 10011).

Preferred substrate materials are polyvinyl (meth)acrylates, polyethylene and polypropylene films and resin-coated papers. In reference to polymers herein, it is intended to include homopolymers as well as copolymers containing recurring units from two or more different polymerizable monomers or segments (in the case of block copolymers).

In general, hydrogels, or water-containing gels, are porous matrices of polymers characterized by hydrophilicity and insolubility in water. In water, they swell to an equilibrium volume but maintain their shape. The hydrophilicity is usually due to the presence of water-solubilizing groups such as hydroxy, carboxy, carbonamido, sulfo and others readily apparent to one skilled in the art attached to the hydrogel polymers. Hydrogel water-insolubility and stability of shape are due to the presence of a three-dimensional network. The swollen state results from a balance between the fluid dispersing forces acting on hydrated chains and cohesive forces that do not prevent the penetration of water into the network. Cohesive forces can be provided by crosslinking. Other forces are electrostatic, hydrophobic or dipole-dipole forces. Further details of hydrogels and their classifications are provided by Kudela in *Encyclopedia of Polymer Science and Engineering*, Volume 7, John Wiley & Sons (New York, 1987), pp. 783-807.

Hydrogels are well known in the medical literature as wound and burn dressings, articles for chemical or drug delivery, conductive articles for electrocardiography, electrophoretic devices and tissue-compatible surgical fillers. We have discovered that some commercial articles used for wound or burn dressings are useful for making rudimentary photochemical delivery articles. Hydrogels known in the art are described for example in U.S. Pat. No. 3,419,006 (King), U.S. Pat. No. 3,664,343 (Assarsson), U.S. Pat. No. 3,993,551 (Assarsson et al), U.S. Pat. No. 5,714,159 (Shalaby), U.S. Pat. No. 5,792,471 (Curatolo), U.S. Pat. No. 4,909,244 (Quarfoot et al) and U.S. Pat. No. 5,115,801 (Cartmell et al), all incorporated herein by reference for their teaching of hydrogels and methods of manufacture. Some of the details of hydrogels are presented herein for illustrative purposes, but it should be understood that the invention is not so limited.

Thus, useful hydrogels can be composed of polymethacrylic esters or polyacrylic esters, polymers derived from hydroxyalkyl methacrylates or acrylates, polyacrylamides or polymethacrylamides with ionic comonomer units, N-vinyl-2-pyrrolidinone copolymers containing less hydrophilic comonomer units or ionizable groups, polymers con-

taining oxyethylene or oxypropylene units (for example polyoxyethylenes, polyoxypropylenes and polyoxyethylene-polypropylenes as described for example in U.S. Pat. Nos. 3,419,006 and 3,664,343) and crosslinked methoxypoly(ethylene glycols). Preferred hydrogels are composed of polymers comprising oxyethylene or polyoxypropylene units or both, and the most preferred hydrogels are composed of polyoxyethylenes.

For example, one useful hydrogel material is derived from the polymerization of poly(ethylene oxide) resin to provide a final weight of 4% PEO resin and 96% water. Such a material is commercially available as 2nd Skin™ Moist Burn Pad burn dressing from Spenco Medical Products. This material has both a backing sheet (substrate) and a cover sheet (on the opposite side of the hydrogel). Another commercially available hydrogel is Vigilon™ wound dressing that is marketed by Bard Medical Division of C. R. Bard Inc. This material appears to be composed of 4% PEO also and has a polyethylene backing sheet on both sides. Of course, at least one of the backing sheets must be removed so the resulting delivery article can imbibe photochemicals and be applied to a processable photographic material.

Preferably, the hydrogel matrix is substantially free of gelatin, gelatin derivatives or other hydrophilic colloidal materials that are commonly used in photographic emulsion layers. Thus, the delivery articles of this invention are different in composition from the processing web described in U.S. Pat. No. 3,179,517 (noted above). In addition, at noted above, the delivery articles of this invention are not "image-donating" or "image-receiving" webs that are generally used in diffusion transfer materials.

The hydrogels can be disposed on the substrates in any suitable fashion. For example, they can be polymerized and cast onto the substrate from the polymerization solution. Alternatively, the hydrogel can be impregnated onto a suitable absorbing, reinforcing material such as a reticulated foam, scrim, or non-woven material and then laminated to the substrate. The substrate is preferably a dimensionally stable backing support. The reinforcing material may be bonded to the dimensionally stable support by means of an adhesive layer or other means prior to impregnation with the hydrogel, or the hydrogel itself may be directly bonded to the support during the casting process or by means of an adhesive.

The various photochemicals necessary to provide a photographic image can be imbibed into or contacted with the hydrogels. Alternatively, the hydrogel matrix can be dried to remove non-chemically bound water to accelerate the uptake of photochemical processing composition upon immersion or direct application. One skilled in the art would readily understand how long the hydrogel needs to be soaked with the photochemical solutions to imbibe the necessary amount of photochemicals. It may vary with the type and amount of photochemicals desired for a given photochemical reaction. The various photochemical solutions are prepared or purchased as described below using the various photochemicals known in the art or from several commercial sources.

In one embodiment, a photochemical released from the photochemical delivery article is a chemical acid or a base. Blocked forms of various photographic reagents can be contained in the photographic material itself, such as a blocked developer that is released upon contact with a chemical base. Upon bringing a chemical base-containing delivery article into reactive association with a silver halide emulsion of such an imagewise exposed photographic material, the chemical base causes the blocked developer to be released and development to occur. A useful chemical

base in this instance would be an aqueous inorganic base, such as an alkali metal hydroxide (for example sodium hydroxide). It is preferred to deliver smaller molecules or ions with the photochemical delivery article in order to increase the rate of diffusion and thereby accelerate photochemical delivery and reaction.

It is appreciated that the hydrogel moisture content, polymer content, crosslinking density, thickness and structural strength can be modified to advantage to suit the processing method for a given photographic material to be processed. The photochemical delivery article should have a hydrogel layer thickness of at least 0.01 mm in order to contain adequate quantities of deliverable photochemical(s) and a thickness of greater than about 0.5 mm is preferred. There is no upper limit on the thickness of the hydrogel layer of the photochemical delivery article, but it is preferred that it be less than about 5 mm. A reinforcing material, if used, can have a matrix or honeycomb structure, random fibers or a fine netting to minimize barriers to solution flow or to make processing more uniform. It is preferred to avoid the use of a reinforcing material in order to minimize barriers to diffusion of photochemical(s).

Lubricants, surfactants, wetting agents or other surface active agents may be included in the hydrogel to improve wetting or swelling of the image photographic materials, photochemical delivery, and lamination and delamination during processing.

#### Black-and-White Image Formation

A black-and-white image can be obtained using the basic photoprocessing steps of black-and-white development and fixing wherein each processing step is carried out using a separate delivery article. Thus, one photochemical delivery article would be used for black-and-white development and a photochemical second delivery article for fixing, each delivery article containing a black-and-white photochemical (for example, a black-and-white developing agent).

For black-and-white image formation, the essential photochemicals that are needed to cause the necessary photochemical reactions are black-and-white developing agents and fixing agents. These and other photochemicals commonly used in black-and-white processing are described below in some detail.

Imaged black-and-white photographic silver halide materials that can be processed can include black-and-white silver halide radiographic films, aerial films, black-and-white motion picture films, duplicating and copy films, and amateur and professional continuous tone black-and-white films and papers. The general composition of such materials is well known in the art.

For example, a black-and-white developing composition can be prepared and imbibed into a hydrogel. This composition can contain one or more black-and-white dihydroxybenzene developing agents, including hydroquinone and derivatives thereof that would be readily apparent to those skilled in the art (see for example, U.S. Pat. No. 4,269,929 of Nothnagle and U.S. Pat. No. 5,457,011 of Lehr et al.). Mixtures of these developing agents can be used if desired.

Other useful developing agents include ascorbic acid and its derivatives are described in a considerable number of publications relating to photographic processes, including U.S. Pat. No. 5,236,816 (Purol et al) and references cited therein. Useful ascorbic acid developing agents include ascorbic acid and the analogues, isomers and derivatives thereof. Such compounds include, but are not limited to, D- or L-ascorbic acid, sugar-type derivatives thereof (such as sorboascorbic acid,  $\gamma$ -lactoascorbic acid, 6-desoxy-L-ascorbic acid, L-rhamnoascorbic acid, imino-6-desoxy-L-

ascorbic acid, glucoascorbic acid, fucoascorbic acid, glucoheptoascorbic acid, maltoascorbic acid, L-arabosaccharic acid), sodium ascorbate, potassium ascorbate, isoascorbic acid (or L-erythroascorbic acid), and salts thereof (such as alkali metal, ammonium or others known in the art), endiol type ascorbic acid, an enaminol type ascorbic acid, a thienol type ascorbic acid, and an enamin-thiol type ascorbic acid, as described for example in U.S. Pat. No. 5,498,511 (Yamashita et al), EP-A-0 585,792 (published Mar. 9, 1994), EP-A-0 573 700 (published Dec. 15, 1993), EP-A-0 588 408 (published Mar. 23, 1994), WO 95/00881 (published Jan. 5, 1995), U.S. Pat. Nos. 5,089,819 and 5,278,035 (both of Knapp), U.S. Pat. No. 5,384,232 (Bishop et al), U.S. Pat. No. 5,376,510 (Parker et al), Japanese Kokai 7-56286 (published Mar. 3, 1995), U.S. Pat. No. 2,688,549 (James et al), U.S. Pat. No. 5,236,816 (noted above) and *Research Disclosure*, publication 37152, March 1995. Mixtures of these developing agents can be used if desired.

The black-and-white developing composition also can include one or more auxiliary co-developing agents that are also well known (for example, Mason, *Photographic Processing Chemistry*, Focal Press, London, 1975). Any auxiliary developing agent can be used, but the 3-pyrazolidone developing agents are preferred (also known as "phenidone" type developing agents). Such compounds are described, for example, in U.S. Pat. No. 5,236,816 (noted above). The most commonly used compounds of this class are 1-phenyl-3-pyrazolidone, 1-phenyl-4,4-dimethyl-3-pyrazolidone, 4-hydroxymethyl-4-methyl-1-phenyl-3-pyrazolidone, 5-phenyl-3-pyrazolidone, 1-p-aminophenyl-4,4-dimethyl-3-pyrazolidone, 1-p-tolyl-4,4-dimethyl-3-pyrazolidone, 1-p-tolyl-4-hydroxymethyl-4-methyl-3-pyrazolidone, and 1-phenyl-4,4-dihydroxymethyl-3-pyrazolidone.

An organic antifogging agent is preferably present in the black-and-white developing composition, either singly or in admixture. Such compounds control the gross fog appearance in the processed elements. Suitable antifoggants include, but are not limited to, benzimidazoles, benzotriazoles, mercaptotetrazoles, indazoles and mercaptothiadiazoles.

The developing composition can also include one or more preservatives or antioxidants. Various conventional black-and-white preservatives can be used including sulfites. A "sulfite" preservative is used herein to mean any sulfur compound that is capable of forming or providing sulfite ions in aqueous alkaline solution.

Various known buffers, such as borates, carbonates and phosphates, can be included in the composition to maintain the desired pH. The pH can be adjusted with a suitable base (such as a hydroxide) or acid. The pH of the developing/fixing composition is generally from about 9 to about 12, and more preferably from about 10 to about 11.

The black-and-white developing composition can contain one or more sequestering agents that typically function to form stable complexes with free metal ions (such as silver ions) in solution, in conventional amounts.

The black-and-white developing composition can also contain other additives including various development restrainers, development accelerators, swelling control agents and stabilizing agents, each in conventional amounts. Examples of such components are described in U.S. Pat. No. 5,236,816 (noted above), U.S. Pat. No. 5,474,879 (Fitterman et al), Japanese Kokai 7-56286 and EP-A-0 585 792.

In the second step of black-and-white processing, a fixing composition containing a photographic fixing agent is used to remove silver. While sulfite ions are present and sometimes acts as a fixing agent, the primary photographic fixing

agents used in the fixing composition are not sulfites. Rather, the useful photographic fixing agents are chosen from thiosulfates (including sodium thiosulfate, ammonium thiosulfate, potassium thiosulfate and others readily known in the art), cysteine (and similar thiol-containing compounds), mercapto-substituted compounds (such as those described by Haist, *Modern Photographic Processing*, John Wiley & Sons, N.Y., 1979), thiocyanates (such as sodium thiocyanate, potassium thiocyanate, ammonium thiocyanate and others readily known in the art), amines and halides. Mixtures of one or more of these classes of fixing agents can be used if desired.

The fixing composition can also include various addenda commonly employed therein, such as buffers, fixing accelerators, sequestering agents, swelling control agents, and stabilizing agents, each in conventional amounts. In its aqueous form, the fixing composition generally has a pH of at least 4, preferably at least 4.5, and generally less than 6, and preferably less than 5.5.

Other details for carrying out black-and-white processing using the delivery articles of this invention would be readily apparent from the teaching provided herein as well as the skill of one experienced in the photographic processing art.

The following TABLE I shows suggested general and preferred (in parentheses) concentrations for essential components of black-and-white processing compositions that would be used to process photographic materials using photochemical delivery articles of this invention. The ranges given in TABLE I have end points that are approximate ("about"). Other components of the processing compositions would be readily apparent to one skilled in the art.

TABLE I

| Processing Step | Essential Photochemical                                         | Concentration (mol/l)   | Contact Time (sec) | Contact Temperature (° C.) |
|-----------------|-----------------------------------------------------------------|-------------------------|--------------------|----------------------------|
| Development     | Developing agent(s): hydroquinones or ascorbic acid derivatives | 0.02-0.5<br>(0.03-0.4)  | 20-480<br>(30-180) | 25-60<br>(35-45)           |
|                 | Co-developing agent(s): substituted pyrazolidinones             | 0-0.05<br>(0.005-0.015) | Same               | Same                       |
|                 | Antioxidant(s): various sulfites                                | 0.1-0.5<br>(0.3-0.4)    | Same               | Same                       |
| Fixing          | Fixing agent(s): thiosulfates                                   | 0.3-2<br>(1-1.5)        | 15-600<br>(20-60)  | 20-60                      |

#### Color Image Formation

Color image formation in various color photographic silver halide materials require certain essential photochemicals including a color developing agent, a photographic bleaching agent and a photographic fixing agent (or both a photographic bleaching and fixing agents). Other useful photochemicals may be needed for various processing methods including, but are not limited to, black-and-white developing agents, co-developing agents, dye stabilizing agents, fixing accelerators, bleaching accelerators, antifoggants, fogging agents and development accelerators. In other instances, the photochemicals may provide a physical benefit such as reduced scumming, reduced crystal growth on processing equipment, reduced sludge, reduced film residue or spotting, storage stability and reduced biogrowth. Examples of such photochemicals include, but are not limited to, surfactants, antioxidants, crystal growth inhibitors and biocides.

Thus, delivery articles can be designed and used for color development, bleaching, fixing (or bleach-fixing), and

optionally a dye stabilizing step. This is generally understood from the conventional Process C-41 processing method for color negative films. Obtaining color positive images in color reversal materials require another unique set of processing steps that are well known in the art (for example, using the conventional Process E-6 or K-25 processing). In addition, obtaining color images in color papers can be achieved using the conventional Process RA steps of color development and bleach-fixing. Motion picture films and prints may include still other processing steps. However, all of these steps and the conventional components of the processing compositions are well known, as described for example, in *Research Disclosure* publication 308119, December 1989, publication 17643, December 1978, and publication 38957, September, 1996. Some additional details are provided below in describing such compositions, but additional details can be supplied from the many publications listed in the noted *Research Disclosure* publications.

Color developing compositions include one or more color developing agents that are well known in the art that, in oxidized form, will react with dye forming color couplers in the processed materials. Such color developing agents include, but are not limited to, aminophenols, p-phenylenediamines (especially N,N-dialkyl-p-phenylenediamines) and others which are well known in the art, such as EP 0 434 097A1 (published Jun. 26, 1991) and EP 0 530 921A1 (published Mar. 10, 1993). It may be useful for the color developing agents to have one or more water-solubilizing groups as are known in the art. Further details of such materials are provided in *Research Disclosure*, publication 38957 (noted above).

In order to protect color developing agents from oxidation, one or more antioxidants are generally included. Either inorganic or organic antioxidants can be used. Many classes of useful antioxidants are known, including but not limited to, sulfites (such as sodium sulfite, potassium sulfite, sodium bisulfite and potassium metabisulfite), hydroxylamine (and derivatives thereof), hydrazines, hydrazides, amino acids, ascorbic acid (and derivatives thereof), hydroxamic acids, aminoketones, mono- and polysaccharides, mono- and polyamines, quaternary ammonium salts, nitroxy radicals, alcohols, and oximes. Mixtures of compounds from the same or different classes of antioxidants can also be used if desired.

Especially useful antioxidants are hydroxylamine derivatives as described for example, in U.S. Pat. No. 4,892,804 (Vincent et al), U.S. Pat. No. 4,876,174 (Ishikawa et al), U.S. Pat. No. 5,354,646 (Kobayashi et al) and U.S. Pat. No. 5,660,974 (Marrese et al), and U.S. Pat. No. 5,646,327 (Burns et al), the disclosures of which are all incorporated herein by reference with respect to antioxidants. Many of these antioxidants are mono- and dialkylhydroxylamines having one or more substituents on one or both alkyl groups. Particularly useful alkyl substituents include sulfo, carboxy, amino, sulfonamido, carbonamido, hydroxy and other solubilizing substituents. One useful hydroxylamine antioxidant is N,N-diethylhydroxylamine.

In other embodiments, the noted hydroxylamine derivatives can be mono- or dialkylhydroxylamines having one or more hydroxy substituents on the one or more alkyl groups. Representative compounds of this type are described for example in U.S. Pat. No. 5,709,982 (Marrese et al), incorporated herein by reference.

It may be desirable to include a chemical base in the color developing composition. Particularly useful chemical bases include inorganic bases such as alkali metal or ammonium

hydroxides (for example sodium hydroxide or potassium hydroxide). Other useful chemical bases are alcoholamines (such as triethanolamine, and diethanolamine).

One or more buffering agents are generally present in the color developing compositions to provide or maintain desired alkaline pH. These buffering agents generally have a pKa of from about 9 to about 13. Such useful buffering agents include, but are not limited to carbonates, borates, tetraborates, glycine salts, triethanolamine, diethanolamine, phosphates and hydroxybenzoates. Alkali metal carbonates (such as sodium carbonate, sodium bicarbonate and potassium carbonate) are preferred. Mixtures of buffering agents can be used if desired.

Polycarboxylic acid or phosphonic acid metal ion sequestering agents are useful in the color developing composition. Such materials are well known in the art, and are described for example in U.S. Pat. No. 4,596,765 (Kurematsu et al) and *Research Disclosure* publications 13410 (June, 1975), 18837 (December, 1979) and 20405 (April, 1981).

It is also possible to include other metal ion sequestering agents (for example, for iron, copper or manganese ion sequestration) in the color developing composition. The composition can also include one or more of a variety of other addenda that are commonly used in photographic color developing compositions, including alkali metal halides (such as potassium chloride, potassium bromide, sodium bromide and sodium iodide), auxiliary co-developing agents (such as phenidone type compounds particularly for black and white developing compositions), antifoggants, development accelerators, wetting agents, fragrances, stain reducing agents, surfactants, defoaming agents, and water-soluble or water-dispersible color dye forming couplers, as would be readily understood by one skilled in the art [see for example, the *Research Disclosure* publications noted above]. The amounts of such additives would be well known to a skilled artisan.

In one embodiment of this invention, a photochemical delivery article consists essentially of a nonporous, dimensionally stable substrate having disposed thereon a poly (ethyleneoxide) hydrogel containing one or more diffusible color development photochemicals.

Color development is generally followed by desilvering using separate bleaching and fixing steps, or a combined bleach/fixing step using suitable silver bleaching and fixing agents. Numerous bleaching agents are known in the art, including hydrogen peroxide and other peracid compounds, persulfates, periodates and ferric ion salts or complexes with polycarboxylic acid chelating ligands. Particularly useful chelating ligands include conventional polyaminopolycarboxylic acids including ethylenediaminetetraacetic acid (EDTA), propylenediaminetetraacetic acid (PDTA) and others described in *Research Disclosure* publication 38957 (noted above), U.S. Pat. No. 5,582,958 (Buchanan et al) and U.S. Pat. No. 5,753,423 (Buongiorno et al). Biodegradable chelating ligands are also desirable because the impact on the environment is reduced. Useful biodegradable chelating ligands include, but are not limited to, iminodiacetic acid or an alkyliminodiacetic acid (such as methyliminodiacetic acid), ethylenediaminedisuccinic acid and similar compounds as described in EP-A-0 532,003, and ethylenediamine monosuccinic acid and similar compounds as described in U.S. Pat. No. 5,691,120 (Wilson et al).

These and many other such complexing ligands known in the art including those described in U.S. Pat. No. 4,839,262 (Schwartz), U.S. Pat. No. 4,921,779 (Cullinan et al), U.S. Pat. No. 5,037,725 (noted above), U.S. Pat. No. 5,061,608 (Foster et al), U.S. Pat. No. 5,334,491 (Foster et al), U.S. Pat.

No. 5,523,195 (Darnon et al), U.S. Pat. No. 5,582,958 (Buchanan et al), U.S. Pat. No. 5,552,264 (noted above), U.S. Pat. No. 5,652,087 (Craver et al), U.S. Pat. No. 5,928,844 (Feeney et al) U.S. Pat. No. 5,652,085 (Wilson et al), U.S. Pat. No. 5,693,456 (Foster et al), U.S. Pat. No. 5,834,170 (Craver et al), and U.S. Pat. No. 5,585,226 (Strickland et al), all incorporated herein by reference for their teaching of bleaching compositions.

Other components of the bleaching solution include buffers, halides, corrosion inhibiting agents, and metal ion sequestering agents. These and other components and conventional amounts are described in the references in the preceding paragraph. The pH of the bleaching composition is generally from about 4 to about 6.5.

Useful fixing agents for photographic fixing compositions are well known. Examples of photographic fixing agents include, but are not limited to, thiosulfates (for example sodium thiosulfate, potassium thiosulfate and ammonium thiosulfate), thiocyanates (for example sodium thiocyanate, potassium thiocyanate and ammonium thiocyanate), thioethers (such as ethylenethioglycolic acid and 3,6-dithia-1,8-octanediol), imides and thiourea.

It is also known to use fixing accelerators in fixing compositions. Representative fixing accelerators include, but are not limited to, ammonium salts, guanidine, ethylenediamine and other amines, quaternary ammonium salts and other amine salts, thiourea, thioethers, thiols and thiolates. Examples of useful thioether fixing accelerators are described in U.S. Pat. No. 5,633,124 (Schmittou et al), incorporated herein for the teaching of fixing compositions. The use of thiocyanate as a fixer accelerator for promoting rapid silver removal is disclosed in U.S. Pat. No. 6,022,676 (Schmittou et al) that is also incorporated herein by reference.

The fixing compositions can also include one or more of various addenda optionally but commonly used in such compositions for various purposes, including hardening agents, preservatives (such as sulfites or bisulfites), metal sequestering agents (such as polycarboxylic acids and organophosphonic acids), buffers, and fixing accelerators. The amounts of such addenda in the working strength compositions would be readily known to one skilled in the art.

The desired pH of the fixing compositions is 8 or less, and can be achieved and maintained using any useful combination of acids and bases, as well as various buffers.

Other details of fixing compositions not explicitly described herein are considered well known in the art, and are described for example, in *Research Disclosure* publication 38957 (noted below), and publications noted therein in paragraph XX(B), U.S. Pat. No. 5,424,176 (Schmittou et al), U.S. Pat. No. 4,839,262 (noted above), U.S. Pat. No. 4,921,779 (noted above), U.S. Pat. No. 5,037,725 (noted above), U.S. Pat. No. 5,523,195 (noted above), U.S. Pat. No. 5,552,264 (noted above), all incorporated herein by reference for their teaching of fixing compositions.

Another photographic processing composition that may be useful is a dye stabilizing composition containing one or more photographic imaging dye stabilizing compounds. Such compositions can be used at the end of the processing sequence (such as for color negative films and color papers), or in another part of the processing sequence (such as between color development and bleaching as a pre-bleaching composition).

Such dye stabilizing compositions generally have a pH of from about 5.5 to about 8, and include a dye stabilization compound (such as an alkali metal formaldehyde bisulfite, hexamethylenetetramine, various benzaldehyde compounds, and various other formaldehyde releasing compounds), buff-

ering agents, bleach-accelerating compounds, secondary amines, preservatives, and metal sequestering agents. All of these compounds and useful amounts are well known in the art, including U.S. Pat. No. 4,839,262 (Schwartz), U.S. Pat. No. 4,921,779 (noted above), U.S. Pat. No. 5,037,725 (noted above), U.S. Pat. No. 5,523,195 (noted above) and U.S. Pat. No. 5,552,264 (noted above), all incorporated herein by reference for their teaching of dye stabilizing compositions.

A preferred dye-stabilizing composition includes sodium formaldehyde bisulfite as a dye stabilizing compound, and thioglycerol as a bleach-accelerating compound. This composition can also be used as a pre-bleaching composition during the processing of color reversal photographic materials.

In some processing methods, a dye stabilizing composition or final rinsing composition is used to clean the processed photographic material as well as to stabilize the color image. Either type of composition generally includes one or more anionic, nonionic, cationic or amphoteric surfactants, and in the case of dye stabilizing compositions, one or more dye stabilizing compounds as described above. Particularly useful dye stabilizing compounds useful in these dye stabilizing compositions are described for example in EP-A-0 530 832 (Koma et al) and U.S. Pat. No. 5,968,716 (McGuckin et al). Other components and their amounts for both dye stabilizing and final rinsing compositions are described in U.S. Pat. No. 5,952,158 (McGuckin et al), U.S. Pat. No. 3,545,970 (Giorgianni et al), U.S. Pat. No. 3,676,136 (Mowrey), U.S. Pat. No. 4,786,583 (Schwartz), U.S. Pat. No. 5,529,890 (McGuckin et al), U.S. Pat. No. 5,578,432 (McGuckin et al), U.S. Pat. 5,534,396 (noted above), U.S. Pat. No. 5,645,980 (McGuckin et al), U.S. Pat. No. 5,667,948 (McGuckin et al), U.S. Pat. No. 5,750,322 (McGuckin et al) and U.S. Pat. No. 5,716,765 (McGuckin et al), all of which are incorporated by reference for their teaching of such compositions.

TABLE II below shows suggested general and preferred (in parentheses) concentrations for essential components of color processing compositions. The ranges given in TABLE II have end points that are approximate ("about"). Other components of the processing compositions would be readily apparent to one skilled in the art.

TABLE II

| Processing Step                       | Essential Photochemical                                   | Concentration (mol/l)    | Contact Time (sec) | Contact Temperature (° C.) |
|---------------------------------------|-----------------------------------------------------------|--------------------------|--------------------|----------------------------|
| Color Development                     | Color developing agent(s):                                | 0.005-0.065 (0.015-0.06) | 30-300 (50-180)    | 30-60 (35-50)              |
|                                       | Antioxidant(s): sulfites or hydroxylamine and derivatives | 0.01-0.1 (0.01-0.05)     | Same               | Same                       |
| Bleaching or Bleach-fixing            | Bleaching agent: ferric poly-carboxylates                 | 0.005-1 (0.1-0.5)        | 10-240 (20-180)    | 25-60                      |
| Fixing or Bleach-fixing               | Fixing agent(s): thiosulfate(s)                           | 0.5-2 (0.8-1.5)          | 20-300 (30-180)    | 25-60                      |
| Dye Stabilizing                       | Dye Stabilizing compound: aldehyde(s)                     | 0-0.05 (0-0.02)          | 0-180 (0-30)       | 25-60                      |
| B & W Developing (for color reversal) | B & W Developing agent: hydroquinones                     | 0.1-0.5 (0.15-0.4)       | 180-500 (300-400)  | 30-60 (35-55)              |
|                                       | Co-developing agent: substituted pyrazolidinone           | 0.001-0.5 (0.005-0.15)   | Same               | Same                       |

As noted above, the compositions described above can be present in photochemical delivery articles and used to pro-

cess black-and-white or color photographic silver halide materials, including but not limited to, black-and-white films and papers, color negative photographic films, color reversal photographic films, and color photographic papers. The general sequence of steps and conditions (times and temperatures) for color photographic processing are well known as Process C-41 (for example, using KODAK FLEXICOLOR photochemicals) and Process ECN-2 for color negative motion films, Process E-6 and Process K-14 for color reversal films, Process ECP for color prints, and Process RA-4 for color papers. Black-and-white photographic processing methods and conditions are also well known (Process RP X-OMAT for radiographic materials processing, Process VERSAMAT 641 or 885 for black-and-white aerial film processing, and Process PROSTAR PLUS for graphic arts film processing).

The photographic materials can be single or multilayer color elements. Multilayer color materials typically contain dye image-forming units sensitive to each of the three primary regions of the visible spectrum. Each unit can be comprised of a single emulsion layer or multiple emulsion layers sensitive to a given region of the spectrum. The layers of the material can be arranged in any of the various orders known in the art. In an alternative format, the emulsions sensitive to each of the three primary regions of the spectrum can be disposed as a single segmented layer. The materials can also contain other conventional layers such as filter layers, interlayers, subbing layers, overcoats and other layers readily apparent to one skilled in the art. A magnetic backing can be included on the backside of conventional supports.

More details of the photographic material structure and components, and suitable methods of processing various types of color elements are described in *Research Disclosure* publication 38957 (noted above). Included within such teachings in the art is the use of various classes of cyan, yellow and magenta color couplers that can be used with the present invention (including pyrazolone and pyrazolotriazole type magenta dye forming couplers).

Thus, a wide variety of types of photographic materials (both black-and-white and color negative and color reversal films and papers, and color motion picture films and prints) containing various types of emulsions can be processed using the present invention, the types of materials being well known in the art (see *Research Disclosure* publication 38957 noted above). The invention can be used to process color photographic papers of all types of emulsions including so-called "high chloride" and "low chloride" type emulsions, and so-called tabular grain emulsions as well.

Representative commercial black-and-white films and papers that are useful in the practice of this invention include, but are not limited to, KODAK T-MAX 400 Film, KODAK TRI-X Pan Film, KODAK VERICHROME PAN Film, KODAK POLYMAX II RC Black and White Papers, KODAK KODABROME II RC F Black and White Paper, KODAK PMAX Art RC V Black and White Paper, KODAK POLYCONTRAST III RC Black and White Paper, KODAK PANALURE Select RC Black and White Paper, KODAK POLYMAX FINE ART Black and White Papers, KODAK AZO Black and White Papers, ILFORD MULTIGRADE IV RC and FB Black and White Papers, ILFORD ILFOBROME GALERIE Black and White Papers, and AGFA MULTICONTRAST CLASSIC and PREMIUM Black and White Papers.

Representative commercial color papers that are useful in the practice of this invention include, but are not limited to, KODAK EKTACOLOR EDGE V, VII and VIII Color

Papers (Eastman Kodak Company), KODAK ROYAL VII Color Papers (Eastman Kodak Company), KODAK PORTRA III, IIIM Color Papers (Eastman Kodak Company), KODAK SUPRA III and IIIM Color Papers (Eastman Kodak Company), KODAK ULTRA III Color Papers (Eastman Kodak Company), FUJI SUPER Color Papers (Fuji Photo Co., FA5, FA7 and FA9), FUJI CRYSTAL ARCHIVE and Type C Color Papers (Fuji Photo Co.), KONICA COLOR QA Color Papers (Konica, Type QA6E and QA7), and AGFA TYPE II and PRESTIGE Color Papers (AGFA). The compositions and constructions of such commercial color photographic materials would be readily determined by one skilled in the art.

KODAK DURATRANS, KODAK DURACLEAR, KODAK EKTAMAX and KODAK DURAFLEX photographic materials and KODAK Digital Paper Type 2976 can also be processed using the present invention.

Representative color negative films that can be processed using the delivery articles of this invention include, but are not limited to, KODAK ROYAL GOLD™ films, KODAK GOLD™ films, KODAK PRO GOLD™ films, KODAK FUNTIME™, KODAK EKTAPRESS PLUS™ films, EASTMAN EXR™ films, KODAK ADVANTIX™ films, FUJI SUPER G Plus films, FUJI SMARTFILM™ products, FUJICOLOR NEXIA™ films, KONICA VX films, KONICA SRG3200 film, 3M SCOTCH™ ATG films, and AGFA HDC and XRS films. Films suitable for processing according to this invention can also be those incorporated into what are known as "one time use cameras".

More preferred color negative films for processing using the apparatus of the present invention are films intended for scanning and electronic image processing rather than optical printing, as described for example in U.S. Ser. No. 09/066,137 filed Apr. 14, 1998 by Sowinski et al and U.S. Pat. No. 6,021,277 (Sowinski et al), the disclosures of which are incorporated herein by reference. The present invention can be used to process a color photographic silver halide material comprised of a blocked but releasable photochemical (such as a blocked but releasable color developing agent). Such a material is disclosed for example in U.S. Ser. No. 09/475,510 filed Dec. 30, 1999 by Irving et al, the disclosure of which is incorporated herein by reference. The photochemical(s) provided by lamination of the photochemical delivery article to a photographic material containing such a releasable, photographically useful chemical can be an chemical acid or a base that releases the blocked photochemical.

The present invention can also be used to process positive color images in color reversal photographic films. The typical sequence of steps includes first development (black-and-white development), reversal processing step, color developing, bleaching, fixing, and stabilizing. There may be various washing steps between other steps, as well as a pre-bleach step or conditioning step before bleaching. Alternatively, dye stabilizing can occur between color developing and bleaching. Many details of such processes are provided in U.S. Pat. No. 5,552,264 (noted above), incorporated herein by reference. Other details are provided in *Research Disclosure*, publication 38957 (noted above), and references noted therein. Useful reversal compositions are described, for example, in U.S. Pat. No. 3,617,282 (Bard et al), U.S. Pat. No. 5,736,302 (Buongiorno et al) and U.S. Pat. No. 5,811,225 (McGuckin et al).

The photochemical delivery articles can be provided in any suitable shape or size. They can be used right after photochemical compositions are imbibed therein, or they can be wound into roll form and stored into a magazine or

cartridge in sealed and protected condition to preserve moisture context and photochemical integrity and activity.

In another embodiment, the photochemical delivery articles can be dehydrated for storage and re-swollen with water or an "activator" solution (such as a basic aqueous solution) at the time of use.

Use of the apparatus of this invention can be achieved by contacting an imagewise exposed photographic material (for example a roll of imaged color negative film, or strips of a certain number of "frames") with the appropriate photochemical delivery articles in their swollen state to form a web laminate. The delivery article is generally brought into reactive association with the silver halide emulsion layer side of the photographic material, not the support side so photochemicals can readily enter the emulsion layer(s) and cause the desired photochemical reactions. Applying liquids such as water, an activator solution, a photochemical processing solution (or its concentrate), or a surfactant or spreading agent solution, or applying pressure may improve the contact and the rate of photochemical delivery and chemical reaction. Such liquids can be added to the delivery article prior to or during contact with the photographic silver halide material. Agitation is not required in the practice of the invention, but sustained pressure, variable kneading, or rolling motions applied to the laminated photographic material and hydrogel can aid the transfer of reagent from the photochemical delivery article.

In one embodiment, the backing substrate that supports the hydrogel is not permanently bonded to the hydrogel and is removed, providing access to the web laminate from the backside of the photochemical delivery article. Thus, water, activator solution, a photoprocessing solution or other aqueous solution can be added to the web laminate at any time during the contact to increase swelling and reaction time. Subsequent capillary action or osmotic pressure at the interface will drive the swelling of the imaged photographic material with the photochemical processing solution in the hydrogel. Concentration gradients of soluble photochemicals will drive exchange between the hydrogel matrix and the contacted photographic material until equilibrium is achieved. Obviously, contact of the delivery article must be to the silver halide emulsion side of the imagewise exposed photographic material. Thus, the silver halide emulsion(s) are in direct contact with the delivery article or in reactive association meaning that the photochemicals can diffuse from the delivery article into the photographic material.

The rate of photochemical delivery and processing can be accelerated by pre-swelling the photographic material with water or an aqueous solution such as a photochemical processing solution or concentrate, or activator solution. The subsequent application of the delivery article by lamination can reduce or eliminate the requirement of a high-precision spreading apparatus for metering a pre-delivered solution for swelling the photographic material. Alternatively, the delivery article can perform as the spreading apparatus when supplemental processing solution is added from the support side of the hydrogel after removal of the substrate.

In some instances, it may be desirable to heat the imagewise exposed photographic material prior to and/or during contact with the photochemical delivery article in order to quicken photochemical reactions or release reactants within the photographic material. This may be especially desirable for processing color photothermographic materials. For the purposes of this invention, photothermographic materials (providing either color or black-and-white images) are considered to be within the definition of "photographic materials" and the photothermographic emulsion layer is considered a "silver halide emulsion layer".

Specific contacting and reaction conditions for various black-and-white and color photoprocessing conditions are provided in TABLES I and II above. However, generally, the contact of photochemical delivery article and imagewise exposed photographic material is for at least 15 seconds, and preferably for from about 30 to about 120 seconds. Processing temperature is at least 25° C., and preferably from about 40 to about 60° C.

In a preferred processing embodiment, water, activator solution or photoprocessing solution is supplied to the web laminate of photochemical delivery article and imaged photographic material to increase the rate of swelling and photochemical reaction (for example color development). This is preferably done somewhat higher than room temperature, for example at from about 40 to about 50° C. After adequate photochemical reaction(s) have occurred, the hydrogel can be pulled away from the processed photographic material and disposed of in a suitable fashion (for example wound into a magazine) or recycled for future reuse (used again to imbibe photochemicals). When a removable supporting substrate is stripped from the photographic material-hydrogel web laminate prior to the completion of the photographic processing (for example in order to add supplemental processing solution), the hydrogel may then be delaminated subsequently with a scraper, blade, or other suitable abrader to mechanically separate them. If the hydrogel was impregnated onto a suitable support mesh or scrim, the hydrogel can still be pulled away from the processed photographic material for storage or disposal as before. The processed photographic material can then be dried and used to provide an image for viewing using conventional procedures or digitization.

The photographic silver halide materials can be scanned immediately after processing with one or more delivery articles or after partial or complete fixing. Preferably, both development and fixing are carried out before scanning.

Once distinguishable images or one or more color records have been formed in the processed photographic materials, conventional techniques can be employed for retrieving the image information for each color record and manipulating the record for subsequent creation of a color balanced viewable image. For example, it is possible to scan a color photographic material successively within the blue, green, and red regions of the spectrum or to incorporate blue, green, and red light within a single scanning beam that is divided and passed through blue, green, and red filters to form separate scanning beams for each color record. If other colors are imagewise present in the material, then appropriately colored light beams are employed. A simple technique is to scan the photographic material point-by-point along a series of laterally offset parallel scan paths. A sensor that converts radiation received into an electrical signal notes the intensity of light passing through the material at a scanning point. Most generally this electronic signal is further manipulated to form a useful electronic record of the image. For example, the electrical signal can be passed through an analog-to-digital converter and sent to a digital computer together with location information required for pixel (point) location within the image. In another embodiment, this electronic signal is encoded with calorimetric or tonal information to form an electronic record that is suitable to allow reconstruction of the image into viewable forms such as computer monitor displayed images, television images, printed images, and so forth.

An image scanner is used to scan an imagewise exposed and photographically processed color negative material delivered from a developing station. As the element is

scanned pixel-by-pixel using an array detector, such as an array charge-coupled device (CCD), or line-by-line using a linear array detector, such as a linear array CCD, a sequence of R, G, and B picture element signals are generated that can be correlated with spatial location information provided from the scanner. Signal intensity and location information can be fed to Digital Image Processor, and the information transformed into an electronic form which can be stored in any convenient storage device or otherwise delivered to the customer by any convenient method.

In one embodiment, it is specifically contemplated to scan a developed image to red, green and blue light to retrieve imagewise recorded information and to scan the same image to infrared light for the purpose of recording the location of non-image imperfections. When such an imperfection or "noise" scan is employed, the signals corresponding to the imperfection can be employed to provide a software correction so as to render the imperfections less noticeable or totally non-noticeable in soft or hard copy form. The hardware, software and technique for achieving this type of imperfection reduction is described by U.S. Pat. No. 5,266,805 (Edgar) and WO 98/31142 (Edgar et al), WO 98/34397 (Edgar et al), WO 99/40729 (Edgar et al) and WO 99/42954 (Edgar et al).

In another embodiment, the developed image can be scanned multiple times by a combination of transmission and reflection scans, optionally in the infrared and the resultant files combined to produce a single file representative of the initial image. Such a procedure is described by U.S. Pat. No. 5,465,155 (Edgar), U.S. Pat. No. 5,519,510 (Edgar), U.S. Pat. No. 5,790,277 (Edgar), U.S. Pat. No. 5,988,896 (Edgar), EP-A-0 944,998, WO 99/43148, WO 99/43149 and WO 99/42954.

Elements having calibration patches derived from one or more patch areas exposed onto a portion of unexposed photographic material as described in U.S. Pat. No. 5,649,260 (Wheeler et al), U.S. Pat. No. 5,563,717 (Koeng et al) and U.S. Pat. No. 5,644,647 (Cosgrove et al) can be usefully employed.

In addition, categorization of the element by an identifying encodement is useful for ensuring that the correct processing parameters are used, as described in copending U.S. Ser. No. 09/456,613, filed Dec. 8, 1999 by Szajewski et al.

Additional illustrative systems for manipulation of digital signals include techniques for maximizing the quality of image records, are disclosed by U.S. Pat. No. 4,553,156 (Bayer), U.S. Pat. No. 4,591,923 (Urabe et al), U.S. Pat. No. 4,631,578 (Sisaki et al), U.S. Pat. No. 4,654,722 (Alkofer), U.S. Pat. No. 4,670,793 (Yamada et al), U.S. Pat. No. 4,694,342 (Klees) and U.S. Pat. No. 4,962,542 (Klees), U.S. Pat. No. 4,805,031 (Powell), U.S. Pat. No. 4,829,370 (Mayne et al), U.S. Pat. No. 4,839,721 (Abdulwahab), U.S. Pat. No. 4,841,361 (Matsunawa et al), U.S. Pat. No. 4,937,662 (Matsunawa et al), U.S. Pat. No. 4,891,713 (Mizukoshi et al), U.S. Pat. No. 4,912,569 (Petilli), U.S. Pat. No. 4,920,501 (Sullivan et al), U.S. Pat. No. 5,070,413 (Sullivan et al), U.S. Pat. No. 4,929,979 (Kimoto et al), U.S. Pat. No. 4,972,256 (Hirosawa et al), U.S. Pat. No. 4,977,521 (Kaplan et al), U.S. Pat. No. 4,979,027 (Sakai et al), U.S. Pat. No. 5,003,494 (Ng), U.S. Pat. No. 5,008,950 (Katayama et al), U.S. Pat. No. 5,065,255 (Kimura et al), U.S. Pat. No. 5,051,842 (Osamu et al), U.S. Pat. No. 5,012,333 (Lee et al), U.S. Pat. No. 5,107,346 (Bowers et al), U.S. Pat. No. 5,105,266 (Telle), U.S. Pat. No. 5,105,469 (MacDonald et al), and U.S. Pat. No. 5,081,692 (Kwon et al). Techniques for color balance adjustments during scanning are disclosed

in U.S. Pat. No. 5,049,984 (Moore et al) and U.S. Pat. No. 5,541,645 (Davis).

Once acquired, the digital color records can be in most instances adjusted to produce a pleasingly color balanced image for viewing and to preserve the color fidelity of the image bearing signals through various transformations or renderings for outputting, either on a monitor or when provided as a color print. A suitable method for color balancing and image processing of electronic image-bearing signals in digital form (density representative electronic signals) is taught in copending U.S. Ser. No. 09/104,548 filed Jun. 25, by Buhr et al, the disclosure of which is incorporated herein by reference (corresponding to EP-A-0 961 482).

Further techniques for transforming image-bearing signals after scanning are disclosed in U.S. Pat. No. 5,267,030 (Giorgianni et al), U.S. Pat. No. 5,528,339 (Buhr et al), U.S. Pat. No. 5,835,627 (Higgins et al), U.S. Pat. No. 5,694,484 (Cottrell et al) and U.S. Pat. No. 5,962,205 (Arakawa et al), the disclosures of all of which are incorporated by reference. Further illustrations of these procedures are provided by Giorgianni and Madden *Digital Color Management*, Addison-Wesley, 1998. The signal transformation techniques disclosed can be further modified so as to deliver an image that incorporates the look selected by a customer.

Matrices and look-up tables (LUTs) can provide useful image transformation. In one embodiment, three 1-dimensional look-up tables can be employed, one for each of a red, green, and blue color record. Due to the complexity of these transformations, it should be noted that the transformation can often be better accomplished by a 3-dimensional LUT. In another embodiment, a multi-dimensional look-up table can be employed, all as described in U.S. Pat. No. 4,941,039 (D'Errico).

In one variation, the R, G, and B image-bearing signals from a transmission scanner are converted to an image metric which corresponds to that from a single reference image-recording device or medium and in which the metric values for all input media correspond to the trichromatic values which would have been formed by the reference device or medium had it captured the original scene under the same conditions under which the input media captured that scene. For example, if the reference image recording medium was chosen to be a specific color negative film, and the intermediary image data metric was chosen to be the measured RGB densities of that reference film, then for an input color negative film, the R, G, and B image-bearing signals from a scanner would be transformed to the R', G', and B' density values corresponding to those of an image which would have been formed by the reference color negative film had it been exposed under the same conditions under which the actual color negative material was exposed.

In another variation, if the reference image recording medium was chosen to be a specific color negative film, and the intermediary image data metric was chosen to be the predetermined R', G', and B' intermediary densities of that reference film, then for an input color negative film according to the invention, the R, G, and B image-bearing signals from a scanner would be transformed to the R', G', and B' intermediary density values corresponding to those of an image which would have been formed by the reference color negative film had it been exposed under the same conditions under which the actual color negative recording material was exposed.

Thus each input film calibrated to be compatible with the present method would yield, insofar as possible, identical intermediary data values corresponding to the R', G', and B' code values required to appropriately reproduce the color image which would have been formed by the reference color negative film on a reference output device. Uncalibrated photographic films may also be used with transformations derived for similar types of films, and the results would be similar to those described.

It is to be appreciated that while the images are in electronic or digital form, the image processing is not limited to the specific manipulations described above. Other useful image manipulation sequences are described by EP-A-0 961,482 (Buhr et al), EP-A-0 961,483 (Buhr et al), EP-A-0 961,484 (Buhr et al), EP-A-0 961,485 (Buhr et al) and EP-A-0 961,486 (Buhr et al), the disclosures of all of which are incorporated by reference. While the images are in digital form, additional image manipulation may be used including, but not limited to, scene balance algorithms (to determine corrections for density and color balance based on the densities of one or more areas within the processed film), tone scale manipulations to amplify film underexposure gamma as described in U.S. Pat. No. 5,134,573 (Goodwin et al), non-adaptive or adaptive sharpening via convolution or unsharp masking, red-eye reduction, and non-adaptive or adaptive grain-suppression. Moreover, the image may be artistically manipulated, zoomed, cropped, and combined with additional images or other manipulations as known in the art. Once the image has been corrected and any additional image processing and manipulation has occurred, the image may be electronically transmitted to a remote location or locally written to a variety of output devices including, but not limited to, silver halide film or paper writers, thermal printers, electrophotographic printers, ink-jet printers, display monitors, CD disks, optical and magnetic electronic signal storage devices, and other types of storage and display devices as known in the art.

It will be appreciated that the output image-bearing signals can be for a reference output device, can be in the form of device-specific code values or can require further adjustment to become device specific code values. Such adjustment may be accomplished by further matrix transformation or 1-dimensional look-up table transformation, or a combination of such transformations to properly prepare the output image-bearing signals for any of the steps of transmitting, storing, printing, or displaying them using the specified device.

The manipulated digital signals (that is, the digital records) can also be forwarded to a suitable output device to provide a display image or stored for future use. The output device may take a number of forms such as a CRT display, CD disk, magnetic devices or other type of storage or output device readily apparent to one skilled in the art.

Besides digital manipulation, the digital images can be used to change physical characteristics of the image, such as "windowing" and "leveling" (used in computed tomography scanning) or other manipulations known in the art.

The apparatus of this invention can be used to process photographic materials in a free-standing, customer accessible kiosk as described for example in EP-A-0 234,833 (Sabbagh), U.S. Pat. No. 5,113,351 (Bostic), U.S. Pat. No. 5,627,016 (Manico) and U.S. Pat. No. 5,664,253 (Meyers).

The invention has been described in detail with particular reference to preferred embodiments thereof, but it will be understood that variations and modifications can be effected within the spirit and scope of the invention.

## PARTS LIST

- 10 camera spool
- 11,13,
- 49, 51 web laminate
- 12 photographic material
- 14,16, 18
- 52, 54, 56 dual guides
- 15, 17, 19,
- 53, 55, 57 roller
- 20 accumulator
- 22, 40 supply reel
- 24, 26,
- 42, 44 take-up reel
- 28 light source
- 30 beam of light
- 32 sensor
- 34, 46 photochemical delivery article
- 36, 48 nonporous substrate
- 38, 50 hydrogel
- 58, 62, 66 Applicator
- 60,64,68 Arrow

We claim:

1. An apparatus for providing a photochemical reaction comprising:
  - a) a means for supplying an imagewise exposed photographic silver halide material comprising at least one silver halide emulsion layer,
  - b) a means for supplying a photochemical delivery article consisting essentially of a nonporous substrate having disposed thereon a hydrogel containing one or more diffusible photochemicals, said nonporous substrate having a thickness of from about 75 to about 200  $\mu\text{m}$ ,
  - c) a means for bringing said imagewise exposed photographic silver halide material and said photochemical delivery article into reactive association to form a web laminate so that a photochemical reaction can occur, and
  - d) a downstream web laminate treating means that is either
    - i) a means for removing said nonporous substrate from said photochemical delivery article in said web laminate, or
    - ii) a means for delaminating said photochemical delivery article from said imagewise exposed photographic silver halide material, and a means for collecting said delaminated photochemical delivery article.
2. The apparatus of claim 1 wherein said nonporous substrate is composed of a resin-coated paper, polyester, cellulosic polymer, polyethylene, polypropylene, polyethylene-polypropylene, polyvinyl chloride, polyvinylidene chloride, polyamide, polyurethane, polyvinyl alcohol, silicone rubber, polyvinyl (meth)acrylate or polystyrene.
3. The apparatus of claim 1 wherein said hydrogel is formed from a polymethacrylic or polyacrylic ester, polyacrylamide or polymethacrylamide, N-vinyl-2-pyrrolidinone copolymer, a polymer containing oxyethylene or oxypropylene units, or a crosslinked methoxypoly(ethylene glycol).
4. The apparatus of claim 1 wherein said hydrogel is free of gelatin, gelatin derivatives or other hydrophilic colloidal materials.
5. The apparatus of claim 1 wherein said photochemical delivery article comprises a black-and-white photochemical, and said imagewise exposed photographic silver halide material is a black-and-white photographic silver halide material.

6. The apparatus of claim 1 wherein said photochemical delivery article comprises a color developing photochemical, and said imagewise exposed photographic silver halide material is a color photographic silver halide material.
7. The apparatus of claim 1 wherein photochemical delivery article is provided in roll form, and said means for supplying it feeds it as a web from said roll form.
8. The apparatus of claim 1 further comprising a means for scanning said web laminate to provide density representative signals.
9. The apparatus of claim 1 further comprising a means for heating said web laminate.
10. The apparatus of claim 1 further comprising a means for applying pressure to said web laminate.
11. The apparatus of claim 1 further comprising a means for applying an aqueous solution to said photochemical delivery article before being carried into said laminating means.
12. The apparatus of claim 11 wherein said applying means is a photochemical processing tank from or through which said photochemical delivery article is supplied.
13. The apparatus of claim 1 further comprising a means for applying an aqueous solution to said imagewise exposed photographic silver halide material prior to being carried into said laminating means.
14. The apparatus of claim 1 comprising said nonporous substrate removing means and a means for applying an aqueous solution to said laminate after said nonporous substrate has been removed.
15. The apparatus of claim 1 that is self-contained.
16. An apparatus for providing a photochemical reaction comprising:
  - a) a means for supplying an imagewise exposed photographic silver halide material comprising at least one silver halide emulsion layer,
  - b) a means for supplying a photochemical delivery article consisting essentially of a nonporous substrate having disposed thereon a hydrogel containing one or more diffusible photochemicals, said nonporous substrate having a thickness of from about 75 to about 200  $\mu\text{m}$ ,
  - c) a means for bringing said imagewise exposed photographic silver halide material and said photochemical delivery article into reactive association to form a web laminate so that a photochemical reaction can occur,
  - d) a means for removing said nonporous substrate from said photochemical delivery article in said web laminate,
  - e) a means for scanning said web laminate to provide density representative signals, and
  - f) a means for delaminating said photochemical delivery article from said imagewise exposed photographic silver halide material.
17. An apparatus for providing a photochemical reaction comprising:
  - a) a means for supplying an imagewise exposed photographic silver halide material comprising at least one silver halide emulsion layer,
  - b) a means for supplying a photochemical delivery article consisting essentially of a nonporous substrate having disposed thereon a hydrogel containing one or more diffusible photochemicals,
  - c) a means for bringing said imagewise exposed photographic silver halide material and said photochemical delivery article into reactive association to form a web laminate so that a photochemical reaction can occur,

- c) a means for contacting said imagewise exposed photographic silver halide material with an aqueous solution prior to its being laminated,
- d) a means for removing said nonporous substrate from said photochemical delivery article in said web laminate,
- d') a means for contacting said web laminate after removal of said nonporous substrate with one or more aqueous solutions,
- e) a means for scanning said laminate to provide density representative signals, and
- f) a means for delaminating said photochemical delivery article from said imagewise exposed photographic silver halide material.

18. An apparatus for providing a photochemical reaction comprising:

- a) a means for supplying an imagewise exposed photographic silver halide material comprising at least one silver halide emulsion layer,
- b) a means for supplying a first photochemical delivery article consisting essentially of a nonporous substrate having disposed thereon a hydrogel containing a first diffusible photochemical,
- c) a means for bringing said imagewise exposed photographic silver halide material and said first photochemical delivery article into reactive association to form a first web laminate so that a first photochemical reaction can occur, and
- d) a means for delaminating said first photochemical delivery article from said imagewise exposed photographic silver halide material,
- e) a means for supplying a second photochemical delivery article consisting essentially of a nonporous substrate having disposed thereon a hydrogel containing a second diffusible photochemical,
- f) a means for bringing said imagewise exposed photographic silver halide material and said second photochemical delivery article into reactive association to form a second web laminate so that a second photochemical reaction can occur.

19. The apparatus of claim 18 further comprising:

- g) a means for delaminating said second photochemical delivery article from said imagewise exposed photographic silver halide material.

20. The apparatus of claim 18 further comprising a means for scanning either said first or second web laminate to provide density representative signals.

21. The apparatus of claim 18 wherein said first and second photochemicals are different.

22. The apparatus of claim 18 further comprising means for heating either said first or second web laminate.

23. The apparatus of claim 18 further comprising a means for contacting either said imagewise exposed photographic silver halide material, said first photochemical delivery article or said second photochemical delivery article with an aqueous solution.

24. An apparatus for providing a photochemical reaction comprising:

- a) a means for supplying an imagewise exposed photographic silver halide material comprising at least one silver halide emulsion layer,
- b) a means for supplying a photochemical delivery article consisting essentially of a nonporous substrate having disposed thereon a hydrogel that is substantially free of diffusible photochemicals, said nonporous substrate having a thickness of from about 75 to about 200  $\mu\text{m}$ ,

- c) a means for bringing said imagewise exposed photographic silver halide material and said photochemical delivery article into reactive association to form a web laminate, and
- d) a means for removing said nonporous substrate from said photochemical delivery article in said web laminate, and
- e) a means for supplying one or more diffusible photochemicals to said photochemical delivery article in said web laminate.

25. An apparatus for providing a photochemical reaction comprising:

- a) a means for supplying an imagewise exposed photographic silver halide material comprising at least one silver halide emulsion layer,
- b) a means for supplying a photochemical delivery article consisting essentially of a nonporous substrate having disposed thereon a hydrogel containing one or more diffusible photochemicals, said nonporous substrate having a thickness of from about 75 to about 200  $\mu\text{m}$ , and
- c) a means for bringing said imagewise exposed photographic silver halide material and said photochemical delivery article into reactive association to form a web laminate so that a photochemical reaction can occur.

26. An apparatus for providing a photochemical reaction comprising:

- a) a means for supplying an imagewise exposed photographic silver halide material comprising at least one silver halide emulsion layer,
- b) a means for supplying a photochemical delivery article consisting essentially of a nonporous substrate having disposed thereon a hydrogel containing one or more diffusible photochemicals, said nonporous substrate having a thickness of from about 75 to about 500  $\mu\text{m}$ ,
- c) a means for bringing said imagewise exposed photographic silver halide material and said photochemical delivery article into reactive association to form a web laminate so that a photochemical reaction can occur, and
- d) a downstream web laminate treating means that is either
  - i) a means for removing said nonporous substrate from said photochemical delivery article in said web laminate, or
  - ii) a means for delaminating said photochemical delivery article from said imagewise exposed photographic silver halide material, and a means for collecting said delaminated photochemical delivery article,

said apparatus further comprising a means for applying an aqueous solution to said imagewise exposed photographic silver halide material prior to being carried into said laminating means.

27. An apparatus for providing a photochemical reaction comprising:

- a) a means for supplying an imagewise exposed photographic silver halide material comprising at least one silver halide emulsion layer,
- b) a means for supplying a photochemical delivery article consisting essentially of a nonporous substrate having disposed thereon a hydrogel containing one or more diffusible photochemicals, said nonporous substrate having a thickness of from about 75 to about 500  $\mu\text{m}$ ,

**29**

- c) a means for bringing said imagewise exposed photographic silver halide material and said photochemical delivery article into reactive association to form a web laminate so that a photochemical reaction can occur, and
- d) a downstream web laminate treating means that is either
  - i) a means for removing said nonporous substrate from said photochemical delivery article in said web laminate, or

5

**30**

- ii) a means for delaminating said photochemical delivery article from said imagewise exposed photographic silver halide material, and a means for collecting said delaminated photochemical delivery article,

- said apparatus further comprising a means for applying an aqueous solution to said laminate after said nonporous substrate has been removed.

\* \* \* \* \*